

Oct. 7, 1924.

1,510,540

A. BRANN

TIPLESS LAMP STEM

Filed June 2, 1921

FIG. 1.



FIG. 2.



INVENTOR  
ALBERT BRANN.

BY  
*J. F. Gobert*  
ATTORNEY

## UNITED STATES PATENT OFFICE.

ALBERT BRANN, OF EAST ORANGE, NEW JERSEY, ASSIGNOR TO WESTINGHOUSE LAMP COMPANY, A CORPORATION OF PENNSYLVANIA.

## TIPLESS LAMP STEM.

Application filed June 2, 1921. Serial No. 474,487.

To all whom it may concern:

Be it known that I, ALBERT BRANN, a citizen of the United States, and a resident of East Orange, in the county of Essex and State of New Jersey, have invented a new and useful Improvement in Tipless Lamp Stems, of which the following is a specification.

This invention relates to the manufacture of stems for incandescent electric lamps of the tipless type.

An object of this invention is to provide a stem composed of several parts or portions of glasses having selected characteristics which permit the portions to be joined or sealed together in a satisfactory and stable manner.

Another and more particular object is to provide a novel stem for an incandescent lamp having an exhaust tube, the inherent characteristic of one of the parts of which differs from a similar characteristic of each of the other parts of the stem, such difference being present to an extent that permits the parts to be joined by sealing in such manner as to avoid excessive strains.

In accordance with the well known practice of manufacturing tipless lamps, an exhaust tube is consolidated with the stem. However, in performing this operation, excessive strains develop in the glass parts of the stem and such strains subsequently produce cracks and breaks, thus rendering the finished lamp useless. This invention, as hereinafter outlined, embodies a novel and satisfactory method of overcoming these defects.

In the accompanying drawings:

Fig. 1 is a side view, partly in section, of the parts of a stem of an incandescent lamp in assembled position; and,

Fig. 2 is a side view of a completed stem, showing an exhaust tube in position and an opening leading from the exterior of the stem to the interior of the exhaust tube.

Referring to the drawings and particularly to Fig. 1, the individual parts or portions of a stem of an incandescent lamp are illustrated as assembled in the usual or overlapped position ready to be heated and pressed together to form a stem. These parts usually consist of a stem or flare tube 5 having a flared portion 6, an arbor 7 for supporting the filament, leading-in con-

ductors 8 and an exhaust tube 9; all of these elements being positioned as illustrated in order that they may be consolidated in the seal formed by pressing the parts together when in plastic condition.

Referring to Fig. 2 a completed stem is shown, with the arbor, flare tube and exhaust tube joined to form a seal. This seal is usually known as the press and is represented in the drawing at 10. An opening or passageway 11 leading from the exhaust tube to the exterior of the stem may be formed directly after the press has been formed and while the glass is still in a plastic condition, by admitting compressed air into the exhaust tube. The passageway 11 allows the air to be exhausted from the lamp bulb after the stem has been sealed therein. The tipping off after the exhaustion of the air is usually performed at a constriction 12 in the exhaust tube. 75

Heretofore, in the manufacture of stems of the general construction illustrated in Fig. 2, it has been found that cracks and breaks develop near the seal and especially at the juncture of the tubes 6 and 9. It has also been found that, without any apparent reason, some of these cracks and breaks develop within a few hours after the formation of the stems and that some of these defects develop during the manufacturing operation of sealing the stems into the bulb. By reason of the development of these defects, a special inspection of the stems before they are assembled in the bulb and another after the stem has been sealed to the bulb, have been necessary. These inspections increase the ultimate cost of the finished product and are to be avoided if possible. 85 90

In the prior construction of lamp stems, the flare and exhaust tubes have been constructed of glasses having substantially the same linear coefficients of expansion. When the exhaust tube is concentrically positioned within the flare tube it is found that, in forming the press, excessive strains are developed, probably due to the unequal cooling as cracks and breaks develop in these stems. 95 100

It would seem that the above mentioned defects are not due to faulty material, rough handling or like causes, but rather from excessive strains produced during the 105

making of the stem which strains subsequently manifest themselves by aging or during subsequent operations.

In endeavoring to overcome the above outlined defects, and bearing in mind that they appear to be due to excessive strains, it is found that, in using glass for the exhaust tube which has a coefficient of expansion differing considerably from that of the 10 glass of the other parts of the stem, a satisfactory union of these parts is obtained when sealed together.

In forming a seal in a stem between glasses having different coefficients of expansion, it is to be noted that the end of the exhaust tube is positioned concentric with the flare tube and expands and contracts during the heating operation, this expansion and contraction being dependent upon the 20 coefficient of expansion of the glass comprising the exhaust tube. This exhaust tube, having a smaller coefficient of expansion than the flare tube, does not expand and contract to the same degree as the flare tube, 25 with the result that, when these parts become cooled after the formation of the press, the exhaust tube apparently is not gripped or placed under such great compression by the flare tube contracting around it and thus 30 affords a means for relieving excessive strains in the glasses composing the parts consolidated at the point of the press.

By employing glass parts having different characteristics, a stem may be constructed 35 which satisfactorily meets the requirements of manufacture. It is, however, to be understood that the degree of variation may be varied by employing glasses of different thickness and by giving full consideration 40 to the positions in which the glasses are held to form seals, as, for example, when one of the parts is to be held concentrically to another of the parts, it must be considered that there will be a pressing of the outer glass 45 upon the inner glass. A satisfactory stem for tipless lamps is obtained by employing a flare tube made of glass having a coefficient of expansion approximating  $.92 \times 10^{-6}$  and an exhaust tube made of glass having 50 a coefficient of expansion varying between  $.83 \times 10^{-6}$  and  $.85 \times 10^{-6}$ .

In forming the seals in the stems of an incandescent lamp by the above described method and by employing glasses which 55 have different characteristics, it is found that the stems may be subjected to a much harder and careless handling than heretofore and that the operators, in handling the stems during the operation of sealing the 60 stems into the bulbs, are not required to exercise great caution. The ability to form the new combination of glasses in order to readily handle and to form the seal between the completed stem and the lamp bulb without 65 the cracking or breaking off of the ex-

haust tube, materially increases the efficiency of the manufacture of incandescent electric lamps and substantially reduces the cost of manufacture.

It is to be understood that various modifications may be made in the stems constructed and in the method of forming the stems, and such modifications are to be included within the scope of this invention as outlined in the following claims.

What is claimed is:

1. A stem for an incandescent lamp of the tipless type comprising a plurality of glass parts, the several parts being of different coefficients of expansion and so disposed when sealed, that the inner portion of the seal will be of a lesser coefficient of expansion than the surface of the seal.

2. A lamp stem comprising leading-in wires, a flare tube and an exhaust tube, said tubes being consolidated in a mass about the leading-in wires, said mass having a lower coefficient of expansion within than on the surface.

3. A stem for an incandescent lamp of the tipless type comprising a flare tube and an exhaust tube sealed thereto, said exhaust tube having a linear coefficient of expansion lower than that of the flare tube.

4. A stem for an incandescent lamp of the tipless type having an exhaust tube constituting a part of the stem, said exhaust tube having a coefficient of expansion considerably lower than the coefficient of expansion of another part of said stem.

5. In a stem construction of an incandescent lamp, the combination of a flare tube, an exhaust tube sealed in a position within said flare tube, the coefficient of expansion of said exhaust tube approximating  $.34 \times 10^{-6}$  and the coefficient of expansion of the flare tube approximating  $.92 \times 10^{-6}$ .

6. In a stem for a tipless incandescent lamp, the combination of a glass tube having one of its ends flared, said glass having a linear coefficient of expansion approximating  $.92 \times 10^{-6}$ , a glass arbor for supporting a lamp filament, leading-in conductors, a glass exhaust tube having a constriction between its ends, said last named glass having a linear coefficient of expansion varying between  $.83 \times 10^{-6}$  and  $.85 \times 10^{-6}$ , said tubes, arbor and conductors being sealed together to form a unit.

7. The method of preventing cracks in lamp stems of the tipless type which comprises providing the component parts of the stem of different coefficients of expansion, disposing a part having the lower coefficient of expansion within another part, heating to render the parts plastic and permitting the parts to cool and unite without setting up detrimental strains by virtue of the difference in their coefficients of expansion.

8. The method of preventing cracks in

lamp stems of the tipless type which comprises providing a flare tube of a given coefficient of expansion and an exhaust tube of a smaller coefficient of expansion, disposing a portion of the exhaust tube within the flare tube, applying heat to render the overlapping portions plastic, permitting the

portions to cool and unite without subsequent cracks by virtue of the difference in degree of their coefficients of expansion. 10

In testimony whereof, I have hereunto subscribed my name this 1st day of June 1921.

ALBERT BRANN.